

Aug. 25, 1942.

H. L. BARTHELEMY ET AL

2,294,154

TREATMENT OF SPINNERETTES TO PREVENT ACCUMULATIONS THEREON

Filed April 25, 1941

Fig. 1

METALLIC SPINNERETTE



Fig. 2.

STAINLESS STEEL BASKET  
CONTAINING SPINNERETTES



INVENTORS

HENRI L. BARTHELEMY  
& GLOVER HOOD ROBINSON  
BY

Pennie, Davis, Marvin & Edmonds  
ATTORNEYS

## UNITED STATES PATENT OFFICE

2,294,154

TREATMENT OF SPINNERETTES TO PRE-  
VENT ACCUMULATIONS THEREONHenri L. Barthelemy and Glover Hood Robinson,  
Rome, Ga., assignors, by mesne assignments, to  
American Enka Corporation, Enka, N. C., a  
corporation of Delaware

Application April 25, 1941, Serial No. 390,334

11 Claims. (Cl. 18—8)

This invention relates to the spinning of viscose rayon and has for its object the provision of certain improvements in spinning apparatus and methods for suppressing the formation of incrustations and craters which form on metallic spinnerettes. It is an object of the invention to provide a method of treating metallic spinnerettes to produce an improved spinnerette as well as an improved arrangement of spinning apparatus for employing the improved spinnerette.

The invention contemplates the treatment of metallic spinnerettes with a cation-active compound to form a thin coating of the compound on the surface of the spinnerette, and particularly that portion thereof immediately surrounding the orifices. The coating of cation-active compound is a very thin film, what may be regarded as a sort of micro-film, and will herein-after, for convenience, be called simply a "film." The invention aims to provide an improved spinning method employing spinnerettes coated with a cation-active compound and the maintenance of a spinning environment which preserves the film in stable attachment on the spinnerette.

We have found that a film of a cation-active compound when applied to a metallic spinnerette will enable the spinnerette to be used in a viscose spin-bath for relatively long periods without the accumulation of incrusting substances near the outer surface of the orifices and which have heretofore formed, especially in spin-baths free of cation-active compounds or rich in zinc sulphate. Spinning operations carried out by using the film coated spinnerettes of the invention will produce, over relatively long periods of time, filaments of uniform normal denier and with practically no minute filaments such as customarily result from the accumulations of solid matter in the form of craters around, and incrustations in, the orifices.

In practices heretofore proposed and also commercially used, cation-active compounds are either mixed with the spinning solution, or dissolved in the spin-bath for the purpose of preventing or suppressing the formation of the craters and incrustations. In the said practices it is necessary to use a relatively large quantity of the cation-active compound in the spinning solution, or in the spin-bath, as the case may be, in order to effect a suppression of the accumulations in and on the spinnerettes. It has been the prevailing belief that the cation-active compounds have a pronounced effect upon the surface tension of the medium in which it is dissolved and

that, as a result thereof, the solid materials which accumulate in the spin-bath, such as precipitated sulphur, salts, complex compounds, etc., do not accumulate in and on the spinnerettes and form the incrustations and craters as they do in the said practices.

As a result of our investigations and discoveries, we have found that a sort of micro-film of a cation-active compound can be caused to form on, or attach itself to, the metallic surface of a spinnerette and that it adheres thereto with a good degree of stability. Moreover, we have discovered that when, for instance, a gold-platinum spinnerette is immersed in any Muller type of spin-bath, the spinnerette acquires a negative charge which varies from about 50 to 300 millivolts. This potential is apparently of sufficient magnitude to prevent too quick a diffusion into the bath of the cation-active compound forming the film. The time of protection afforded is about 15 to 20 days. We have found that a film of the cation-active compound may be formed on the metallic surface of spinnerettes by treating the spinnerettes with an aqueous solution of a cation-active compound under conditions which eliminate the air layer on the metallic surface and permit the film to form thereon. A very effective method of accomplishing the removal of the gas film and forming the film of cation-active compound is to treat the spinnerettes in a boiling aqueous solution of the cation-active compound for about fifteen minutes. However, fair results can also be obtained by performing the same treatment in hot or lukewarm solutions, preferably with the help of a small difference of electrical potential to promote the migration of the cation to the spinnerette.

The optimum concentration of cation-active material in water is determined by systematic tests, as cation-active compounds found on the market exhibit different activities, and as experience taught us there exists for each one an optimum concentration above which spinning stability is impaired again.

The invention in its more or less complete aspects contemplates the provision of an improved spinning method which comprises employing a metallic spinnerette coated with a film of a cation-active compound under conditions causing the spinnerette to be under a negative electrical potential. In spinning viscose rayon in accordance with the invention, the liquid environment in contact with the spinnerette is kept substantially free of anion-active compounds or other like materials or conditions tending to

displace or inhibit the cation-active compound from its stable attachment to the spinnerette.

In the accompanying drawing:

Fig. 1 is a side view of a metallic spinnerette having a film of a cation-active compound on its surface, and

Fig. 2 is a diagrammatic illustration of apparatus which may be used in a method of the invention.

In practicing the invention for producing a spinnerette coated with a film of cation-active compound, a metallic spinnerette, especially one formed of noble metal, for example a spinnerette formed of an alloy containing approximately seventy percent (70%) of gold and thirty percent (30%) of platinum, is thoroughly cleaned to remove adhering solid and liquid matter. The cleaned spinnerette is submerged in a solution comprising, for example, approximately two grams of lauryl pyridinium chloride in one liter of distilled water. The solution is boiled for a sufficient length of time to eliminate surface gases, about fifteen minutes being ordinarily suitable to accomplish this purpose. As the film of gas is removed from the surface of the spinnerette, the cation-active compound attaches itself to the surface of the spinnerette in the form of a film which seems to have the characteristics of a micro-film. In applying the film of cation-active compound to a metallic spinnerette in the apparatus illustrated in Fig. 2, an aqueous solution of a cation-active compound, like lauryl pyridinium chloride, is heated in the basin until it becomes warm or hot and a small difference of electrical potential is applied to the spinnerette by means of the battery, to promote the migration of the cations to the spinnerette.

The spinnerette coated with the cation-active compound is removed from the solution and is thereafter dried in any suitable manner to remove the water, due precautions being taken not to disturb or injure the film. A satisfactory manner of removing the water is accomplished by heating the spinnerette in a ventilated drier at a temperature not exceeding 65° C.

The coated spinnerette is attached to the spinning apparatus in the usual way, care being taken not to touch or otherwise disturb the film on the surface of the spinnerette in the immediate vicinity of the orifices. The film not only covers the large surfaces of the spinnerette, but seems to cover and coat the walls of the orifices themselves. The film appears to prevent wetting of the spinnerette by the spin-bath and also wetting of the insides of the orifices by the viscose solution. So long as the spinnerette is under a negative potential and the spin-bath substantially free of anion-active compounds, the film on the surface of the spinnerette remains in stable or firm adherence notwithstanding the solubility in the aqueous spin-bath of the cation-active compound forming the film.

While many cation-active compounds are suitable for the purposes of this invention, we have found that lauryl pyridinium chloride, cetyl pyridinium bromide (sold by du Pont under the trade name "Fixanol"), and a product sold by Carbide and Carbon Chemicals Corporation under its trade name "Amine 22L" are desirable because of their effectiveness and availability.

Spinnerettes formed of the noble metals, for example gold, platinum and palladium and alloys thereof, have negative potentials when in the presence of acid spinning baths and may be used in the apparatus and method of the invention.

Spinnerettes formed of tantalum may likewise be used.

In the usual viscose spinning operation, and particularly in those operations which employ relatively large quantities of zinc sulphate in the spin-bath, the orifices of the metallic spinnerettes become incrusted with solid matter of indefinite composition, which also frequently forms craters around the orifices. These incrustations and/or craters obstruct the free passage of spinning solution through the orifices, causing what is known as "slow holes." These slow holes cause the filaments to be much smaller in diameter than they would normally be. These incrustations and craters form at such a rapid rate that the spinnerettes must be subjected to frequent inspection, for example once every forty-eight hours, to keep them in operating condition. Inspection includes removing the spinnerettes from the spin-bath, rubbing the surface with the thumb to remove the craters and seeing whether the flow from any of the holes appears sluggish. If the flow is sluggish, the spinnerette must be dismounted and replaced. When, however, the spinnerettes are coated with a film of a cation-active compound according to the invention, they may be operated continuously for a week or more without inspection and without producing any appreciable quantity of minute filaments.

The invention not only eliminates the necessity of contaminating the viscose and the spin-bath with a cation-active compound in order to eliminate incrustations and craters, but it also reduces the quantity of the compound necessary for the purpose to almost an immeasurably small quantity.

We claim:

1. A metallic spinnerette comprising a film of a cation-active compound in stable attachment on the surface of the metal.
2. Apparatus for the spinning of viscose which comprises a metallic spinnerette having a film of a cation-active compound, and means for maintaining said spinnerette under a negative electrical potential during spinning.
3. The method of treating a metallic spinnerette which comprises cleaning the spinnerette to remove solid or liquid matter, submerging the cleaned spinnerette in a hot solution of a cation-active compound for a sufficient time to permit the cation-active compound to displace gas from the surface of the spinnerette and to form thereon a film of the cation-active compound.
4. The method of treating a metallic spinnerette which comprises heating the spinnerette in an aqueous solution of a cation-active compound for a sufficient time to form a film of the cation-active compound on the surface of the spinnerette.
5. The method of treating a metallic spinnerette which comprises submerging the spinnerette in a boiling aqueous solution of a cation-active compound for a sufficient time to form a film of the cation-active compound on the surface of the spinnerette, removing the spinnerette from the solution, and evaporating water from the surface of the spinnerette.
6. In a method of spinning viscose, the improvement which comprises employing a metallic spinnerette having in stable attachment on its surface a film of a cation-active compound, maintaining the spinnerette under a negative electrical potential, and maintaining the liquid environment in contact with the spinnerette suf-

ficiently free of anion-active compounds to maintain the film of cation-active compound for a relatively long period.

7. In a method of spinning viscose, the improvement which comprises applying a film of a cation-active compound on the spinnerette, placing the spinnerette in the spin-bath, and maintaining the spinnerette under a negative electrical potential and the spin-bath free of anion-active compounds that will displace the said film.

8. A spinnerette formed of a noble metal comprising a film of a cation-active compound in stable attachment on the surface of the metal.

9. Apparatus for the spinning of viscose which comprises a spinnerette formed of a noble metal having a film of a cation-active compound, and means for maintaining said spinnerette under a negative electrical potential during spinning.

10. In a method of spinning viscose, the im-

provement which comprises employing a spinnerette formed of a noble metal having in stable attachment on its surface a film of a cation-active compound, maintaining the spinnerette under a negative electrical potential, and maintaining the liquid environment in contact with the spinnerette sufficiently free of anion-active compounds to maintain the film of cation-active compound for a relatively long period.

11. The method of treating a metallic spinnerette which comprises placing the spinnerette in an aqueous solution of a cation-active compound, placing the spinnerette under a negative electrical potential to promote the migration of the cation to the spinnerette and forming a film of the cation-active compound thereon.

HENRI L. BARTHELEMY.  
GLOVER HOOD ROBINSON.